



US006272753B2

(12) **United States Patent**  
**Packer**

(10) **Patent No.:** **US 6,272,753 B2**  
(b4) **Date of Patent:** **\*Aug. 14, 2001**

(54) **MULTI-LAYER, MULTI-GRADE MULTIPLE CUTTING SURFACE PDC CUTTER**

(75) Inventor: **Scott M. Packer**, Pleasant Grove, UT (US)

(73) Assignee: **Smith International, Inc.**, Houston, TX (US)

(\*) Notice: This patent issued on a continued prosecution application filed under 37 CFR 1.53(d), and is subject to the twenty year patent term provisions of 35 U.S.C. 154(a)(2).

Subject to any disclaimer, the term of this patent is extended or adjusted under 35 U.S.C. 154(b) by 0 days.

(21) Appl. No.: **09/410,954**

(22) Filed: **Sep. 27, 1999**

**Related U.S. Application Data**

(62) Division of application No. 08/869,781, filed on Jun. 5, 1997, now Pat. No. 5,979,578.

(51) **Int. Cl.<sup>7</sup>** ..... **E21B 10/46**

(52) **U.S. Cl.** ..... **30/108.2; 175/434**

(58) **Field of Search** ..... **76/108.2, DIG. 12, 76/108.1; 175/428, 430, 431, 432, 434**

(56) **References Cited**

**U.S. PATENT DOCUMENTS**

|           |        |                |       |         |
|-----------|--------|----------------|-------|---------|
| 4,225,322 | 9/1980 | Knemeyer       | ..... | 51/295  |
| 4,255,165 | 3/1981 | Dennis et al.  | ..... | 51/309  |
| 4,339,009 | 7/1982 | Busby          | ..... | 175/374 |
| 4,592,433 | 6/1986 | Dennis         | ..... | 175/329 |
| 4,604,106 | 8/1986 | Hall et al.    | ..... | 51/293  |
| 4,743,515 | 5/1988 | Fischer et al. | ..... | 428/698 |

|           |         |                    |       |           |
|-----------|---------|--------------------|-------|-----------|
| 4,823,892 | 4/1989  | Fuller             | ..... | 175/329   |
| 4,984,642 | 1/1991  | Renard et al.      | ..... | 175/329   |
| 5,031,484 | 7/1991  | Packer             | ..... | 76/108.6  |
| 5,119,714 | 6/1992  | Scott et al.       | ..... | 76/108.2  |
| 5,172,778 | 12/1992 | Tibbitts et al.    | ..... | 175/420.1 |
| 5,205,684 | 4/1993  | Meskin et al.      | ..... | 408/145   |
| 5,217,081 | 6/1993  | Waldenström et al. | ..... | 175/420.2 |
| 5,238,074 | 8/1993  | Tibbitts et al.    | ..... | 175/428   |
| 5,248,006 | 9/1993  | Scott et al.       | ..... | 175/420.2 |
| 5,335,738 | 8/1994  | Waldenström et al. | ..... | 175/420.2 |
| 5,351,770 | 10/1994 | Cawthorne et al.   | ..... | 175/374   |
| 5,351,772 | 10/1994 | Smith              | ..... | 175/428   |
| 5,379,853 | 1/1995  | Lockwood et al.    | ..... | 175/428   |
| 5,431,239 | 7/1995  | Tibbitts et al.    | ..... | 175/428   |
| 5,467,669 | 11/1995 | Stroud             | ..... | 76/108.2  |
| 5,492,188 | 2/1996  | Smith et al.       | ..... | 175/432   |
| 5,499,688 | 3/1996  | Dennis             | ..... | 175/426   |
| 5,667,028 | 9/1997  | Truax et al.       | ..... | 175/428   |
| 5,722,499 | 3/1998  | Nguyen et al.      | ..... | 175/431   |

**FOREIGN PATENT DOCUMENTS**

|           |         |      |   |
|-----------|---------|------|---|
| 0 156 264 | 10/1985 | (EP) | . |
| 0 177 466 | 4/1986  | (EP) | . |
| 2 190 412 | 11/1987 | (GB) | . |
| 2 204 625 | 11/1988 | (GB) | . |

*Primary Examiner*—Douglas D. Watts

(74) *Attorney, Agent, or Firm*—Christie, Parker & Hale, LLP

(57) **ABSTRACT**

An improved polycrystalline diamond composite (“PDC”) cutter with secondary PDC cutting surfaces in addition to a primary PDC cutting surface is formed comprising of at least two wafers of cemented carbide bonded together. The secondary cutting surfaces are formed by compacting and sintering diamond in grooves formed at the surface of the wafers. Wafers of different grades of cemented carbide may be used. Moreover, different grades of diamond may be compacted and sintered in different grooves.

**16 Claims, 4 Drawing Sheets**



*FIG. 1**FIG. 2A*

*FIG. 2B**FIG. 2C*

*FIG. 3A**FIG. 3D**FIG. 3B**FIG. 4**FIG. 3C**FIG. 5*

*FIG. 6*

## MULTI-LAYER, MULTI-GRADE MULTIPLE CUTTING SURFACE PDC CUTTER

### CROSS REFERENCE TO RELATED APPLICATION

This application is a divisional of patent application Ser. No. 08/869,781, filed Jun. 5, 1997 is now U.S. Pat. No. 5,979,578.

### BACKGROUND OF THE INVENTION

The present invention relates to polycrystalline diamond composite ("PDC") cutters with multiple cutting surfaces used in drag bits for drilling bore holes in earth formations.

PDC cutters have a cemented carbide body and are typically cylindrical in shape. The primary cutting surface of the cutter is formed by sintering a PDC layer to a face of the cutter. Secondary cutting surfaces are formed on the cutter body by packing grooves formed on the cutter surface with diamond and then sintering the diamond to form polycrystalline diamond cutting surfaces.

The cutters are inserted on a drag bit outer body exposing at least a portion of the cutter body and the diamond cutting surface. Typically, the cutter makes contact with a formation at an angle, i.e., the diamond cutting layer is at an angle to the formation surface. As the bit rotates, the PDC cutting layer edge makes contact and "cuts" away at the formation. At the same time portions of the exposed cutter body also make contact with the formation surface. This contact erodes the cutter body surrounding the secondary cutting surfaces, revealing a secondary surface cutting edge or wear surface.

One preferable way to prolong the life of a cutter during drilling, is to increase the hardness of the substrate forming the cutter body. The increase in hardness tends to provide a stiffer or more rigid support for the PDC cutting surface. This will help reduce the magnitude of the tensile stresses in the PDC cutting surface induced by a bending moment during the cutting action, thereby reducing the frequency of cracks in the PDC layer which run perpendicular to the interface. However, a stiffer, harder substrate typically has a lower fracture toughness value and in some cases a lower transverse rupture strength. As a result, once a crack is initiated in the PDC, the substrate is unable to slow the propagation. If a crack is allowed to propagate, it can cause the cutter to fracture and fail catastrophically resulting in the eventual failure of the bit.

Accordingly, there is a need for a cutter having secondary cutting surfaces with an increased resistance to breakage. Moreover, there is a need for a cutter having a stiff, hard substrate supporting the cutter cutting layer for improved cutting but which prevents the propagation of crack growth through the cutter body.

### SUMMARY OF THE INVENTION

The present invention is an improved polycrystalline diamond composite ("PDC") cutter having multiple cutting surfaces and a body which is composed of at least two grades of carbide; and a method for making the same. In a preferred embodiment, a cutter body or substrate is formed from layers of carbides. For descriptive purposes, the substrate layers are also referred to as "wafers." Each wafer has a top end, a bottom end and a body therebetween.

The cutter body is formed by bonding the wafers of cemented carbide together, one on top of the other. It is preferred that a stiffer grade cemented carbide is used to form the uppermost portion of the cutter which interfaces

with the primary PDC cutting layer. A stiffer substrate provides better support for the cutting layer which results in enhanced cutting.

Secondary cutting surfaces are formed by compacting and sintering diamond in grooves formed on the body surface of the wafers. The grooves preferably span the length of the wafers. The grooves can be of any shape. Generally, the shape and orientation of the grooves is dictated by the formations to be cut. In addition, the orientation of the grooves, and hence, of the secondary cutting surfaces, may be varied by rotating the wafers in relation to each other. For example, the wafers may be oriented such that the grooves on their surfaces are aligned for forming grooves that are continuous between the wafers. Moreover, different grades of diamond may be compacted and sintered in different grooves.

### BRIEF DESCRIPTION OF THE DRAWINGS

FIG. 1 is an isometric view of a PDC cutter with secondary cutting surfaces.

FIG. 2A is an isometric view of five cemented carbide wafers, three of which having grooves, which when bonded form the PDC cutter body of FIG. 1.

FIG. 2B is an isometric view of a PDC cutter uppermost wafer having a non-planar surface for bonding the PDC layer.

FIG. 2C is an isometric view of a PDC cutter wafer having a groove having a non-smooth surface.

FIG. 3A is an isometric view of a PDC cutter having curve shaped secondary cutting surfaces.

FIG. 3B is an isometric view of a PDC cutter having square shaped secondary cutting surfaces.

FIG. 3C is an isometric view of a PDC cutter having inverted "V" shaped secondary cutting surfaces.

FIG. 3D is an isometric view of a PDC cutter having skewed arc shaped secondary cutting surfaces.

FIG. 4 is an isometric view of a PDC cutter formed from four cemented carbide wafers where the grooves on the wafers are aligned to form continuous grooves along the cutter body.

FIG. 5 is an isometric view of a PDC cutter with a plurality of square shaped secondary cutting surfaces oriented in a helical pattern.

FIG. 6 is an isometric view of a PDC cutter having a PDC layer having a non-planar cutting surface.

### DETAILED DESCRIPTION OF THE PREFERRED EMBODIMENT

Generally, PDC cutters have a carbide body 10 having a cylindrical shape with a cutting face 12 (FIG. 1). A PDC layer 14 is sintered on the cutting face of the body (FIG. 1). While the present invention is described herein based on a cylindrical-shaped cutter, the invention is equally applicable to other shapes of cutters.

The body of the PDC cutter is formed by bonding together at least two cemented carbide wafers 16. The wafers are preferably cylindrical having a top 18 and bottom 20 end and a body having a circumferential outer surface therebetween (FIG. 2A). To form the cutter body, the wafers are preferably stacked one on top of the other and bonded.

A primary cutting surface is formed by sintering a PDC layer 14 on the top end of the uppermost wafer 22 (i.e., the top end of the cutter). The uppermost wafer may have a non-planar uppermost surface 13 (e.g., a surface having

irregularities formed on it) forming the cutting face of the body onto which is bonded the PDC layer (FIG. 2B). A non-planar cutting face provides for a greater area for bonding the PDC layer. In addition, the non-planar face provides for more a gradual transition from the carbide to the diamond. Consequently, the shift in the coefficient of thermal expansion from the carbide to the diamond is also made more gradual. As a result, the magnitude of the stresses generated on the interface between the PDC layer and the carbide are reduced. To form the PDC layer, typically, diamond is spread over the surface and sintered in a high temperature, high pressure press to form polycrystalline diamond. The outer diamond surface 15 may also be non-planar as shown in FIG. 6.

Additional cutting surfaces 24 (referred herein as "secondary" cutting surfaces) are formed on the cutter body. To form the secondary cutting or wear surfaces, grooves 26 are formed on the wafer circumferential outer surface. Preferably, the grooves span the full length of the wafers. The grooves may have irregular (e.g., wavy) surfaces 27 (FIG. 2C). Grooves having an irregular surface provide a greater area for bonding the diamond material. Moreover, the irregular surfaces provide for more a gradual transition from the carbide to the diamond. Consequently, the shift in the coefficient of thermal expansion from the carbide to the diamond is also made more gradual. As a result, the magnitude of the stresses generated on the interface between the diamond and the carbide are reduced.

Grooves which span the full length of the wafer are easier to form since the groove can begin and end at an end face 18, 20 of a wafer. As a result, the grooves have maximum depth from their onset.

The process of forming the grooves and the subsequent process of compacting and sintering polycrystalline diamond in these grooves is known in the art. Typically, the sintering occurs in a high temperature, high pressure press. For example, U.S. Pat. No. 5,031,484 describes a process for fabricating helically fluted end mills with PDC cutting surfaces by sintering and compacting polycrystalline diamond in helically formed grooves in fluted end mills. Generally speaking, the grooves for polycrystalline diamond have a half round cross section without sharp corners. Typically a groove may be 0.060 inch wide and 0.050 inch deep.

The secondary cutting surface shape is driven by the shape of the groove on which it is formed. Secondary cutting surfaces can be in the shape of rings, arcs, dots, triangles, rectangles, squares (FIG. 3B). Moreover, they can be in the shape of an inverted "V" (FIG. 3C), they can be longitudinal, circumferential, curved (FIG. 3A) or skewed (FIG. 3D). The shapes of the cutting surfaces that can be formed is basically unlimited. A combination of cutting surface shapes may be incorporated in single wafer or a single cutter body.

Furthermore, the groove (and secondary cutting surface) orientation may be varied by rotating the wafers in relation to each other prior to bonding. For example, the wafers may be aligned such that the grooves are aligned forming a continuous groove 30 that are between the wafers 16 (FIG. 4). The secondary cutting surfaces can be oriented along the cutter body, as necessary, to accommodate the task at hand. For example, the secondary cutting surfaces can be oriented in a helical pattern along the length of the cutter (FIG. 5).

Moreover, the cutting surfaces can be arranged on the cutter body so as to vector the cutting forces applied by the cutter as needed for the cutting to be accomplished.

Additionally, grooves, and thereby secondary cutting surfaces, of various shapes may be formed in a single wafer. Similarly, each wafer may have grooves of different shapes.

The carbide wafers can be made of different grades of cemented carbide. For example, a stiff (i.e., hard) substrate is desired to support the primary PDC cutting layer so as to prevent breakage of the PDC layer. However, with a stiff, hard substrate some toughness may be sacrificed. As a result, cracks forming at the cutting face 15 of the primary PDC cutting layer may propagate through the length of the substrate resulting in the splitting of the substrate and failure of the cutter.

To alleviate this problem and to provide the desired stiffness for prolonging the life of the PDC cutting layer and for enhancing its cutting performance, at least a wafer made from stiff cemented carbide and a wafer made from tough cemented carbide are bonded to form the substrate (body) of the cutter. A harder stiffer carbide may include an average particle size of less than 4 microns and a cobalt content of 12% by weight or less. A tougher grade of carbide will exceed these values. The toughness and hardness of the carbide is also a function of the binder material used (e.g., Ti, Co, Ni) as well as the weight % and/or the constituents of eta phase that make up the carbide. Moreover, the toughness and hardness of the carbide material may vary from supplier to supplier.

The stiffer cemented carbide wafer forms the top of the cutter for supporting the primary PDC cutting layer. The tougher cemented carbide wafer is bonded to the stiffer wafer to form the lower portion of the cutter body. The stiffer wafer provides the desired support to the PDC layer. The tougher cemented carbide wafer which is not as prone to cracking as the stiffer wafer, serves as a crack arrestor. Thus, a crack that propagates through the stiffer wafer should be arrested once it reaches the tougher wafer, preventing the failure of the cutter.

As it will become apparent to one skilled in the art, multiple wafers of various grades of cemented tungsten carbides, dual phase ("DP") carbides such as carbides with high volume % eta phase, ceramic metals commonly referred to as "cermets" or other carbides may be used to form cutters tailored to the task at hand. By varying the grade and type of the cemented carbide, the peak stress magnitude on the cutter may be decreased and the stress distribution along the cutter body may be optimized so as to yield a cutter with an enhanced operating life. In addition, each secondary cutting surface may be formed from different grades of diamond to optimize the cutting efficiency of the cutter.

Since the grooves formed on the wafers can have a full depth at their onset, the cutting surfaces formed within such grooves will have a full thickness throughout their length. Consequently, as the substrate around a secondary cutting surface wears, a cutting surface of significant thickness will always be exposed reducing the risk of cutter cracking or breakage.

The present invention, therefore, provides a modular approach to cutter design. The approach allows for the formation of a cutter with various shapes of secondary cutting surfaces, with secondary cutting surfaces of different diamond grades, and with substrates of multiple grades of cemented carbide, allowing for the optimization of the stress distribution within the cutter and for the vectoring of cutting forces applied by the cutter which result in enhanced cutter performance and life.

In a preferred embodiment, the wafers are stacked together, the grooves are compacted with the appropriate

grade of diamond, and diamond is spread on the top end of the uppermost wafer, forming an assembly. The assembly is then pressed together under high temperature, high pressure, bonding the wafers together and forming a cutter body and sintering the diamond to form a PDC layer in the cutter body top end and secondary PDC cutting surfaces on the grooves. After pressing, the carbide may be ground away, exposing additional portions of the secondary cutting surfaces to allow for enhanced cutting.

In alternate embodiment, the wafers are diffusion bonded together to form the cutter body such as by HIPing. In yet a further embodiment the wafers are brazed together using conventional methods. As it would be apparent to one skilled in the art, the wafers may be bonded with any of the aforementioned methods prior or after the compacting and sintering of the diamond material in the grooves. Similarly, the primary PDC cutting layer may be sintered prior or after the bonding of the wafers.

In another embodiment, the wafers used may be in a green state prior to bonding with the other wafers or prior to the sintering of the PDC material. Is such a case, the wafers themselves are sintered during the bonding process or during the sintering of the PDC process.

Having now described the invention as required by the patent statutes, those skilled in the art will recognize modifications and substitutions to the elements of the embodiment disclosed herein. For example, a secondary cutting surface may be employed on a cylindrical compact brazed to a cutter stud as used in some types of rock bits. Such modifications and substitutions are within the scope of the present invention as defined in the following claims.

What is claimed is:

1. A method for forming a PDC cutter comprising the steps of:

forming a plurality of carbide wafers having a pair of opposite end faces and a body therebetween, each wafer having a length;

forming a groove in a circumferential surface of a wafer; bonding the wafers to each other at their end faces

forming a cutter body wherein one of the wafer end faces forms the cutter body primary cutting end face; and

bonding polycrystalline diamond in the groove for forming a secondary cutting surface.

2. A method as recited in claim 1 wherein the step of forming a groove comprises the step of forming a groove having an irregular surface.

3. A method as recited in claim 1 further comprising the step of forming a non-planar surface on the end face of the wafer forming the primary cutting end face.

4. A method as recited in claim 1 wherein the step of bonding polycrystalline diamond in the groove comprises the steps of:

compacting diamond particles in the groove; and  
pressing the wafer with diamond particles in a high temperature high pressure press for forming a polycrystalline diamond cutting surface.

5. A method as recited in claim 1 further comprising the step of bonding a layer of polycrystalline diamond on the body primary cutting end face for forming a primary cutting surface.

6. A method as recited in claim 5 further comprising the step of forming a non-planar outer surface on the polycrystalline diamond layer.

7. A method as recited in claim 5 wherein the step of bonding a layer comprises the step of bonding a layer of polycrystalline diamond on end face of a wafer prior to the step of bonding the wafers.

8. A method as recited in claim 1 wherein the steps of bonding the polycrystalline diamond and bonding the wafer comprise the steps of:

compacting diamond particles in the groove; and  
pressing the wafers and the compacted diamond in the groove in a high temperature, high pressure press for forming a cutter body with a polycrystalline diamond cutting surface in the groove.

9. A method as recited in claim 1 wherein the pressing step further comprises the step of simultaneously pressing a layer of diamond material applied to the wafer end forming the body primary cutting end face for forming a primary diamond cutting surface on the PDC cutter body.

10. A method as recited in claim 1 wherein the step of forming a groove comprises the step of forming a groove that spans the length of the wafer.

11. A method as recited in claim 1 wherein the step of forming a groove further comprises the step of forming a second groove on the circumferential surface of the wafer having the first groove, and wherein the bonding step comprises the step of bonding a first grade of diamond in one groove and bonding a second grade of diamond in the second groove.

12. A method as recited in claim 1 wherein the step of forming a groove comprises the step of forming a groove on at least two wafers.

13. A method as recited in claim 12 wherein the step of bonding the wafers further comprises the step of helically orienting the grooves in said at least two wafers relative to each other prior to bonding.

14. A method as recited in claim 1 further comprising the step of grinding a portion of the cemented carbide around the secondary cutting surface to expose an additional portion of the secondary cutting surface.

15. A method as recited in claim 1 wherein the step of forming a plurality of carbide wafers comprises the step of forming at least one carbide wafer from the material selected from the group consisting essentially of dual phase carbides and cermets.

16. A method as recited in claim 1 wherein the step of forming a plurality of carbide wafers comprises the step of forming at least one wafer with a binder selected from the materials consisting essentially of Ti, Co and Ni.